

Patented Mar. 1, 1932

1,847,326

# UNITED STATES PATENT OFFICE

LEWIS L. ALSTED, OF APPLETON, WISCONSIN

PAPER PULP AND PROCESS OF MAKING SAME

No Drawing.

Application filed January 28, 1928. Serial No. 250,343.

This invention relates to a new article of commerce, namely, dry mechanical or ground wood pulp susceptible of ready, quick and economic re-pulping for subsequent use in the manufacture of paper, board, or other fibrous products and to improved processes for the production and manufacture thereof.

Due to the ease and low cost of production, its light color, excellent printing qualities, et cetera, ground wood or so-called mechanical pulp forms an important constituent in the manufacture of many forms and grades of paper. It forms about 80% of the pulp stock used in the manufacture of newsprint paper and from 85 to 95% of the pulp stock from which the cheaper grades of so-called wall paper are made, and it forms the major constituent in the manufacture of various and sundry other types and grades of paper. Its importance in the industry is, therefore, great and as will be appreciated the cost to the consumer of paper containing ground wood pulp is largely influenced by and dependent upon the cost to the paper manufacturer of such pulp.

As is well known in the art, very few species of wood can be used in the manufacture of a satisfactory ground wood pulp. In years gone by when these species were plentiful in certain sections of this country, many paper mills were built in locations accessible not only to this wood supply but also to the paper markets. There was no occasion for long hauls of the raw materials. The pulp was produced at the paper mill from raw material obtained close by and from the pulp the paper stock was prepared and paper produced all in a substantially continuous process or operation. These were ideal conditions from the manufacturing standpoint and the paper was produced at the lowest possible cost. Under this order of things, however, the raw material supply became removed farther and farther from the paper mill, occasioning added costs due to the gradually increasing distances the material had to be hauled or transported.

These conditions have persisted for many years with the result that today the supplies of these species of wood which are relied

upon in the manufacture of ground wood pulp are situated at great distances from most of the mills in this country. This means that in order to do business in face of the competition now offered for instance by the Canadian paper mills located at or near a source of supply and therefore enjoying the ideal manufacturing conditions which formerly obtained in this country, the mills in this country, manufacturers of newsprint paper in particular, are compelled to do business on such a small margin that many of them have been forced to shut down, and it is generally believed that unless relief is shortly forthcoming, it is only a question of time before the others will be forced to do likewise.

In order to operate under present conditions, the newsprint mills in this country must either have the raw material shipped to them over long distances or else purchase prepared ground wood pulp in the form now commercially obtainable from pulp mills situated at or near a source of supply. The first is out of the question in the manufacture of newsprint paper and other papers containing a high percentage of ground wood as the freight and other costs incident to the hauling and handling of the raw material would run the cost of the paper above present market prices, and the second, also chiefly because of the freight consideration, is not, from a sound business point of view, feasible in competition with paper made at or near the source of supply, because of the fact that ground wood pulp as now manufactured must be kept in a wet condition from the time it is made until it is used at the paper mill and for that reason it is necessary to ship approximately from one to two tons of water in the pulp for every ton of pulp. This of course necessitates the payment of freight charges two or three times greater than would be required for the net amount of pulp present in any shipment and constitutes a very heavy burden on the paper manufacturer.

It has long been realized that a great saving in the cost of paper having a high ground wood content could be effected if the pulp could be dried to atmospheric dryness, or sub-

stantially so, before shipment, without deter-  
ring or preventing subsequent re-pulping at  
the paper mill. Many have tried to dry  
ground wood pulp and ship it in that condi-  
tion and the literature in the industry con-  
tains many articles on the subject with some  
few accounts of methods advanced for ac-  
complishing the desired end. In addition,  
I have personal knowledge of several unsuc-  
cessful commercial attempts to manufacture  
dry ground wood pulp.

However, in spite of a full realization in  
the industry of the need for and advantages  
which would be attendant upon the commer-  
cial manufacture and sale of dry mechanical  
pulp and of the various attempts as recorded  
in the literature pertaining to the industry  
and of the actual commercial attempts to  
which I have referred, I am not aware of a  
single practical or successful solution of the  
problem nor am I aware of ground wood pulp  
ever having been treated or manufactured in  
such form that it could be thoroughly dried  
and subsequently, readily, quickly, economi-  
cally and thoroughly re-pulped and returned  
to its original pulp condition such as is neces-  
sary before it can be used in the manufacture  
of satisfactory paper at the paper mill.

It has been found and is well known  
throughout the industry that ground wood  
pulp dried before use in paper making will  
not come back or re-pulp to its original con-  
dition on wetting in the beater or otherwise  
and with the employment of any reasonable  
amount of treatment the paper made there-  
from is marred by small lumps of pulp  
formed of little dry sections or pockets in the  
pulp mass which do not and will not break  
down or separate satisfactorily during the  
re-pulping operation. Ground wood pulp is  
made by a purely mechanical grinding oper-  
ation in which substantially none of the in-  
ter-cellular matter is destroyed or removed.  
This inter-cellular matter includes resinous  
binding substances which become inter-  
spersed or distributed throughout the ground  
wood, and in any attempt to dry the resultant  
pulp, there is a decided tendency for fibers to  
compact or consolidate and due to the pres-  
ence of this inter-cellular matter, fibers be-  
come glued or bound together in a mass which  
is more or less impervious to moisture and not  
susceptible of being broken down or having  
its fibers satisfactorily separated in a beater  
or any other apparatus, such as would be  
used in the re-pulping operation. It is for  
these reasons that it has heretofore been  
necessary to ship the ground wood in a wet  
condition in the form of blankets or laps  
containing approximately from 50 to 60, and  
even 75, percent of moisture.

One object of my invention is to provide  
as an article of commerce dry ground wood  
pulp which may be manufactured at a raw  
material mill located at a source of the neces-

sary species of wood and shipped any dis-  
tance to a paper mill and which will have  
the property of being capable of ready, eco-  
nomical and complete re-pulping in the  
manufacture of paper.

Another object of my invention is to pro-  
vide improved processes for the treatment  
and manufacture of ground wood pulp so  
that it may be completely dried, or dried to  
atmospheric dryness, and left in that condi-  
tion indefinitely or for any length of time  
required and which may be readily, quickly  
and economically re-pulped and returned to  
its original pulp condition.

A further object of the invention is to pro-  
vide as a new article of commerce a dry pulp  
mixture containing predetermined percent-  
ages of ground wood and sulphite or other  
chemical pulp, the mixture being susceptible  
of thorough and complete re-pulping at the  
paper mill and the immediate manufacture  
therefrom of paper, newsprint for instance,  
without the addition of any other pulp or  
other ingredients to the mixture.

In view of the conditions existing in the  
industry, as previously described, the ad-  
vantages of the above will be apparent and  
it is ventured that the resultant savings to the  
paper mills of this country, particularly  
manufacturers of paper having a high ground  
wood content such as newsprint paper, will  
enable such mills either to continue or reopen  
operations in face of the competition referred  
to and on a basis which will net them a fair  
return on the amount of capital invested.

I shall now proceed to a disclosure of sev-  
eral processes as illustrative embodiments of  
my invention.

I have discovered that by adding a small  
amount, say 20% of sulphite or other chemi-  
cal pulp or cellulose fibers to ground wood,  
the resultant pulp may be dried to substan-  
tially atmospheric dryness and yet be capable  
of easy, quick and economic re-pulping with-  
out the appearance of specks or lumps, either  
in the re-pulped mass or in the resultant  
paper, such as invariably occur in the pulp  
and paper resulting from untreated ground  
wood which has been dried. In carrying out  
this process, I provide a suitable mixing tank  
into which the given quantities of the ground  
wood and chemical or other cellulose pulp,  
each preferably in slush form, may be con-  
veyed. Suitable agitating means may be  
used to advantage in the mixing tank for stir-  
ring the two pulps so as to produce a thorough  
and uniform mixture. I then convey the  
mixture to a lap or web forming apparatus  
(wet machine) of any of the well known  
types, such apparatus usually including a  
tank into which the slush pulp is flowed, and  
a perforated suction cylinder or drum which  
revolves in the tank partly submerged in the  
pulp so as to cause the latter to be deposited  
free of a large percentage of its water on the

outer surface of the drum or cylinder. The pulp in any well known manner may be stripped from this cylinder in a continuous web or sheet and conveyed on the usual endless belt or apron between press rolls and delivered either in sheets or so-called noodle-like fragments such as would result in well known manner from the use of a doctor or similar device in conjunction with one of the 5 press rolls. As the pulp, free of a large percentage of the water issues from the press rolls of the wet machine, it may be conveyed either to a shredding machine where the sheets or fragments are shredded and then through a 10 suitable drying tunnel or other drying apparatus or direct to a drying apparatus. It is preferred to dry the pulp to atmospheric dryness, or substantially so, after which it is ready for shipment or for storage. The resultant dry pulp product may be either in the 15 form of shredded fragments or pieces such as would result from the use of a shredder previous to the drying step, or it may be in the form of the larger noodle-like fragments, such as would result from passing the pieces 20 of pulp which would result from doctoring the pulp from one of the press rolls direct to the drying apparatus, or it may be in the form of a rolled sheet if the pulp is taken from the 25 wet machine in a continuous web or sheet and passed as such through the drying apparatus, or it may be in the form of regular shaped sections of appreciable size, say of an area of 1 to 4 square feet or larger, such as would result 30 by cutting the web or sheet before or after it leaves the wet machine into sections of the desired shape and size and then passing such sections through the drying apparatus, or such as would result from passing 35 the continuous web or sheet through the drying apparatus and then severing or cutting the dried sheet into sections of the desired shape and size.

It will be appreciated from the above that 40 the process described is characterized chiefly by the mixing of a given amount, say 80%, of ground wood pulp in slush form with a given amount, say 20%, of chemical pulp such as sulphite or other cellulose fiber pulp in 45 slush form and subsequently removing the water therefrom and drying the pulp to substantially atmospheric dryness for shipment or storage. It will also be appreciated that in carrying out the process I am in no way 50 limited or restricted to any particular type or types of apparatus which may be employed. The art abounds in various forms of apparatus suitable for carrying out each step of the process and a choice of any of these is 55 of course within the contemplation of the invention. Neither is it desired to limit or restrict the process in any way to the particular percentages mentioned of ground wood and chemical pulp. Twenty percent of the 60 chemical or other cellulose fiber pulp has been

found in actual tests to give very satisfactory results. Other percentages, however, will also give satisfactory results, and from a commercial standpoint, it may be desirable to keep the percentage of chemical pulp down 70 as low as may be consistent with good results so that the resultant product will be universally usable throughout the paper making industry in the manufacture of all ground wood content papers.

So far as I am aware, ground wood is seldom, if ever, used alone in the manufacture of paper or paper products. A paper might be made of all ground wood content, but it would be so inferior and lacking in strength 75 that it would be of no practical utility. From 15 to 50% of sulphite or other chemical pulp or cellulose fiber is usually mixed with the ground wood by the paper manufacturer to give strength to the paper. Standard newsprint paper embodies about 20% sulphite pulp and 80% ground wood. Therefore, for the newsprint paper mills ground wood pulp to which had been added 20% of sulphite 80 pulp would be the ideal mixture, because the dried product could then be re-pulped at the paper mill and made directly into paper without the addition of any other materials. Board and some of the cheaper grades of wall paper, however, contain as low as 15% and 85 possibly less of sulphite or other chemical pulp or cellulose fiber and it may be desirable in commercial use of the invention to manufacture a separate grade of dry ground wood 90 pulp containing less than 20% chemical pulp, 95 say 15% or even 10%, for paper mills manufacturing paper or board with an 85% or 90% ground wood content.

However, tests and experiments which I have conducted indicate that the addition of only 15% or less of the chemical pulp to the ground wood does not give as satisfactory a product as the 20% mixture, but I have further discovered that by adding a small percentage, 4 to 6%, for instance, of colloidal clay, such as bentonite, to mixtures of ground wood and chemical pulp in which the percentage of the latter is so small as to render the mixture otherwise inferior to the more desirable 80% ground wood—20% sulphite 100 mixture, the conditions are greatly improved, resulting in a product fully as good, if not better, than the mixture comprising merely 80% ground wood and 20% sulphite. The latter mixture, however, has been found to be 105 entirely satisfactory for re-pulping after drying and it is not necessary to add a colloidal substance, or any other material, to such a mixture. The percentage of chemical pulp in such a mixture may be reduced slightly 110 below 20% and there appears to be no limit in the other direction. In other words, the chemical pulp in percentages anywhere from 20 to 50%, or greater, could be used in the 115 mixture with entirely satisfactory results.

In mixtures where the chemical pulp constitutes appreciably less than 20%, I add, as above pointed out, a small percentage of a colloidal substance, such as bentonite, which 5 I have found renders such mixtures capable of easy and quick re-pulping after they have been dried.

I have further discovered that by mixing 10 with ground wood pulp a small percentage of colloidal clay, such as bentonite, without the addition of chemical pulp or any other material, the ground wood pulp may be thoroughly dried for shipment or storage and that it may subsequently be easily re-pulped preparatory 15 to the manufacture of paper. In this connection I have found that from 6 to 8% of bentonite gives very satisfactory results, although I do not desire to be limited to these exact percentages. The bentonite or 20 clay seems to have the effect of preserving an even distribution of the pitch, albumen and other inter-cellular and water resistant substances in the ground wood, so that after it has been dried and subsequently immersed in 25 water, it will wet and absorb evenly without forming the dry water resistant sections or pockets previously described in connection with ordinary ground wood.

When using bentonite in my processes, I 30 prefer to prepare it as follows:—

A portion of this material in its natural state, usually in a hard dry semi-rock like form is broken up and then ground or otherwise reduced to a finely divided condition.

35 It is then mixed with water and in this form added in the proper percentage to the pulp while the latter is still in slush form. If desired the bentonite may be ground or otherwise finely divided directly in water or it may 40 be added in a dry finely divided form directly to the pulp slush.

According to my processes, as above set forth, it will be appreciated that I am enabled to produce as an article of commerce 45 dried paper pulp comprising either ground wood alone or ground wood with varying percentages of sulphite or other chemical pulp or cellulose fiber and that in the case of the ground wood and chemical pulp mixtures the 50 percentages may be accurately determined and controlled.

The addition of sulphite or other cellulose fiber and/or a colloidal substance such as bentonite, in small quantity to the ground wood 55 prior to drying will in no way have any injurious effect upon the resultant pulp or paper. On the other hand, it is in fact an advantage in that it may be the means of shipping to a paper mill a dry pulp mixture 60 which may be directly made into paper or board of its specifications without the addition of any other pulp, fiber, or other materials. Furthermore, the mixture according to the present invention being effected with 65 the pulps in slush form, it is entirely feasible

to control the exact percentages desired with predetermined accuracy, which is also a substantial advantage in the dry pulp.

Just why the addition of a small amount of chemical pulp or other cellulose fiber to the ground wood with or without a small amount of colloidal clay, or the addition of a small percentage of colloidal clay alone prevents the ground wood from compacting, consolidating and adhering or the fibers thereof becoming glued together in a wood-like mass approximating its original natural condition is not known, but actual tests and experiments have shown conclusively that such action is thereby overcome and the ground wood preserved in such condition that it may be quickly, economically and thoroughly re-pulped and worked up in standard beating equipment at the paper mill and satisfactory paper or board products produced therefrom. The 70 chemical or cellulose fibers seem to act as canals to conduct water into every portion of the dried pulp and it consequently absorbs water quickly and evenly without the formation of sections or pockets of dry pulp as is the case with sheets, flakes or fragments made up entirely of ground wood, while a colloidal substances such as bentonite seems to have the 75 property of effecting and preserving an even distribution of the pitch, albumen and other inter-cellular and water resistant substances in the ground wood so that after the pulp has been dried it will, when immersed in water, wet, absorb and break down quickly and easily into its original pulp condition.

Pulp manufactured according to any of the above processes may be produced in any desired form including the various forms above named—shredded, creped, continuous rolled sheets, regular shaped sections of appreciable area, or fragments such as would result from the use of a doctor or scraper in conjunction with one of the press rolls of the wet machine. The pulp in shredded, creped, or similar form, may be conveniently baled or bundled for shipment while the pulp, if in uniform sections of appreciable area, may be suitably stacked and wired or otherwise tied into bundles of desired size or weight.

It is not desired nor intended that the several processes I have described above shall in any manner limit or restrict my invention, as such processes have been set forth as merely illustrative embodiments of the same. In the above and in the appended claims, I wish it to be understood that the term "sulphite" is intended to comprehend any pulp or fibre that is substantially free of the inter-cellular resinous binding materials, such as any chemical pulp or cellulose fiber and that where the term "bentonite" is employed it is intended that the same be construed to include any colloidal clay or substance such as silica gel, aluminum hydroxide, and et cetera. In its 115 120 125 130

- brodest aspects, my invention contemplates all of these various materials and/or their equivalents used either alone or in combination in the manufacture of dry pulp, the basic 5 feature of the invention residing in the mixing with ground wood pulp any substance having the property of rendering said pulp, when dry, uniformly pervious to water and readily returnable to its original pulp condition. The invention also contemplates, as a new article of commerce, the resultant pulp product having the characteristics and properties above pointed out regardless of how the same may be produced or manufactured.
- 10 15 The invention claimed is:
1. A process for the manufacture of dry mechanical pulp, consisting in first preparing ground wood in slush form, then mixing therewith a substance capable of entering 20 into a final product made from the pulp having the property of rendering said pulp, when dry, uniformly pervious to water and readily returnable to its original pulp condition, and then drying the pulp to substantially 25 atmospheric dryness.
  2. A process for the manufacture of dry pulp for subsequent re-pulping in the manufacture of paper, board and other fibrous products, consisting in first preparing ground 30 wood in slush form, then preparing chemical pulp in slush form, mixing the two together in definite proportions while in such form, and then drying to substantially atmospheric dryness.
  3. As a new article of commerce, a dry pulp mixture containing substantially 80% ground wood and substantially 20% chemical pulp.
  4. As a new article of commerce, a dry pulp mixture containing ground wood and substantially resin-free pulp.
  5. As a new article of commerce, a dry mechanical pulp containing ground wood and a colloidal clay.
  6. As a new article of commerce, a dry pulp mixture containing ground wood and sulphite.
  7. As a new article of commerce, a dry mechanical pulp containing ground wood and a small percentage of bentonite.
  8. As a new article of commerce, a dry pulp mixture containing ground wood, a chemical pulp and a colloidal clay.
  9. As a new article of commerce, a dry pulp mixture containing substantially 80% ground wood and substantially 20% sulphite.
  10. As a new article of commerce, dry ground wood pulp containing a substance capable of entering into a final product made 60 from the pulp having the property of rendering said pulp, when dry, uniformly pervious to water and readily returnable to its original pulp condition.
  11. A process for the manufacture of dry pulp for subsequent re-pulping in the manu-
- ture of paper, board and other fibrous products, consisting in preparing ground wood in slush form, then adding thereto a small percentage of bentonite in finely divided form and evenly distributing the same 70 throughout the pulp, and then drying the pulp to substantially atmospheric dryness.
12. A process for the manufacture of dry pulp for subsequent re-pulping in the manufacture of paper, board and other fibrous products, consisting in first preparing ground wood in slush form, then preparing a chemical pulp in slush form, mixing the two together in definite proportions while in such form and adding a small percentage of a colloidal clay in finely divided form, and then drying the pulp to substantially atmospheric dryness. 75
13. As a new article of commerce, a dry pulp susceptible of quick and economic re-pulping in the manufacture of paper, board and other fibrous products, comprising ground wood and a highly absorbent resin-free fibrous substance which acts to conduct water quickly and evenly throughout the 80 pulp when the latter is subjected to the re-pulping operation. 85
14. As a new article of commerce, a dry pulp susceptible of quick and economic re-pulping in the manufacture of paper, board and other fibrous products, comprising ground wood and a colloidal substance having a property of effecting and preserving an even distribution of the pitch, albumen and other inter-cellular substances in the ground 90 wood so that the pulp when subjected to the re-pulping operation will wet, absorb and break down quickly and easily into its original pulp condition. 95
15. As a new article of commerce, a dry pulp susceptible of quick and economic re-pulping in the manufacture of paper, board and other fibrous products, comprising ground wood, highly absorbent cellulose fibers, and a colloidal substance in finely 100 divided form, the latter having the property of effecting and preserving an even distribution of the pitch, albumen and other inter-cellular matter present in the ground wood and the fibrous material having the property 105 of quickly and evenly conducting water throughout the pulp when the latter is subjected to the re-pulping operation. 110
16. A process for the manufacture of pulp which may be completely dried and subsequently re-pulped in the manufacture of paper, board and other fibrous products, which process consists first in preparing ground wood in slush form, then preparing 115 chemical pulp in slush form, then mixing the two in approximately the proportion of four parts ground wood to one part substantially resin-free chemical pulp, then partly removing the water from said mixture, and 120
- 130

then drying to substantially atmospheric dryness.

17. As a new article of commerce, an air dry pulp mixture containing ground wood and cellulose fiber, the cellulose fiber being thoroughly interspersed with the ground wood fiber to prevent interadhesion between the wood fibers.

In witness whereof, I hereto affix my signature.

**LEWIS L. ALSTED.**

**30**

**35**

**40**

**45**

**50**

**55**

**60**

**65**